

## UNITED STATES PATENT OFFICE

2,169,193

## CHROMIUM-TITANIUM-SILICON ALLOY

George F. Comstock, Niagara Falls, N. Y., assignor to The Titanium Alloy Manufacturing Company, New York, N. Y., a corporation of Maine

No Drawing. Application January 6, 1938,  
Serial No. 183,583

## 4 Claims. (Cl. 75—134)

My invention consists of the formation of a new and improved alloy for adding titanium to cast iron along with the addition of chromium at the same time with the titanium.

5 The advantages of adding these two elements of titanium and chromium together to cast iron were described in U. S. Patent No. 1,955,791 granted to me April 24, 1934, but heretofore it was necessary as set forth in my patent to make 10 these additions by means of two separate ferro-alloys, since no combined alloy of chromium and titanium was known that was practical for use in cast iron at ordinary foundry temperatures.

My new alloy is practical for this purpose, since 15 it also contains silicon in an amount properly related to the chromium and titanium contents therein so as to promote ready solubility in the molten cast iron. The iron content of my new alloy is therefore necessarily low, and the carbon 20 content is also low for the same reason that the silicon content is high, in order to confer suitable fusibility and solubility in the molten iron.

Obviously it is more convenient and advantageous to add the two alloying elements of chromium and titanium to cast iron by a single low- 25 iron alloy, than by the use of two separate ferro-alloys, which latter practice involves the addition of so much more cold material to the molten iron after it has left the furnace. My new alloy also 30 has an advantage over the grade of ferro-chromium now generally used for cast iron in that its carbon content is low, so that the chromium added by my new alloy is not already combined with carbon, but such chromium is more free to 35 distribute itself through the matrix of the iron homogeneously instead of as isolated particles of chromium carbide.

Up to the present time my new combined alloy 40 of titanium and chromium has been made with its approximate composition within the following limits:

|                        | Percent        |
|------------------------|----------------|
| Titanium               | 10.65 to 29.55 |
| Chromium               | 14.52 to 41.69 |
| Iron                   | 7.42 to 21.73  |
| Silicon and impurities | 26.28 to 46.07 |

Iron and other impurities are derived chiefly from the ores of titanium and chromium used in making the alloy, and may include up to 5% 50 manganese, 3% aluminum, and 1% each of magnesium, zirconium, nitrogen, carbon, etc.

Permissible ranges of composition of this new and improved alloy may therefore within the scope of my invention be set as follows, with a 55 satisfactory average analysis about as indicated:

|                  | Permissible | Average |
|------------------|-------------|---------|
| Titanium         | Percent     | Percent |
| Chromium         | 10 to 30    | 20      |
| Iron             | 15 to 45    | 30      |
| Silicon          | 0 to 25     | 12      |
| Carbon           | 20 to 45    | 35      |
| Aluminum         | 0 to 1      | 0.4     |
| Other impurities | 0 to 3      | 1.0     |
|                  | 0 to 5      | 1.6     |

10 The preferred analysis of course would be one showing no iron, carbon, aluminum, or other impurities, but this is practically impossible of attainment at a reasonable cost because of the lack of purity of the ores which must be used in commercial practice.

15 My new alloy may be made in the usual type of single-phase carbon-lined electric furnace such as is used for making ferro-titanium.

The following example will show one practical 20 method of manufacture of this alloy.

An intimate mixture of 150 lbs. of granular rutile, 175 lbs. of chrome ore, 165 lbs. of 90% ferro-silicon, and 30 lbs. of sodium chlorate was 25 first prepared. The rutile contained about 92.5%  $TiO_2$ , 4%  $ZrO_2$ , 2.7%  $SiO_2$  and 0.22%  $Fe_2O_3$ , and was crushed so that 98% passed through a —80 mesh screen. The chrome ore was crushed finer than 20 mesh and contained about 54.8%  $Cr_2O_3$ , 14%  $FeO$ , 4.5%  $SiO_2$ , with the balance alumina, 30 magnesia, etc. The ferro-silicon, containing less than 10% iron, was crushed through a 20 mesh screen.

This mixture was charged gradually for about 35 an hour into a hot electric furnace with a 16 in. square carbon electrode, operating at 50 volts and about 10,000 amperes. About 10 minutes after the charge was completely added, the furnace was tapped into a cast iron mold, and the alloy and slag were allowed to cool. When cold 40 the slag was separated, and 202 lbs. of this new alloy was recovered, containing approximately 20.62% titanium, 26.71% chromium, 12.42% iron, and 40.25% silicon plus impurities.

A higher-grade alloy could readily be made 45 by using a higher-grade chrome ore, containing a lower percentage of  $FeO$ . It is also possible to make my new alloy by a slight modification of the method disclosed in my U. S. Letters Patent No. 1,946,670 dated February 13, 1934, 50 the change required being a substitution of high-grade chrome ore for a suitable proportion of the titanium ore in the charge. This method, however, does not involve the use of high-grade ferro-silicon, and hence is more economical of 55

materials, but requires a longer period of operation of the furnace to reduce the necessary silicon from its ore.

In the production of my new alloy by the 5 method just described in the example, a uniform stock of the following analysis was accumulated:—

|                                 | Per cent |
|---------------------------------|----------|
| Titanium                        | 22.8     |
| 10 Chromium                     | 26.9     |
| Silicon                         | 34.42    |
| Iron                            | 14.06    |
| Aluminum                        | 1.01     |
| Zirconium                       | 0.13     |
| 15 Carbon                       | 0.40     |
| Other impurities (Mg, Mn, etc.) | 0.28     |
|                                 | —        |
|                                 | 100.00   |

This alloy was used to treat some gray cast 20 iron melted in a foundry cupola, the amount of the addition of my new alloy being 1% of the weight of the iron.

Comparative results of tests of the original and 25 treated iron are set forth in the following table:

|    | Kind of iron                                 | Plain<br>gray iron<br>untreated | Same iron<br>plus 1%<br>FeTi | Same iron<br>plus 1%<br>CrTiSi |
|----|----------------------------------------------|---------------------------------|------------------------------|--------------------------------|
| 30 | Carbon content                               | 3.38                            | 3.36                         | 3.39                           |
|    | Silicon content                              | 2.41                            | 2.52                         | 2.63                           |
|    | Titanium content                             |                                 | 0.098                        | 0.128                          |
|    | Chromium content                             |                                 |                              | 0.23                           |
|    | Transverse strength, lbs. per<br>1.25" diam. | 3,980                           | 4,070                        | 4,365                          |
|    | Deflection, in. on 12 in. span               | 0.12                            | 0.11                         | 0.105                          |
| 35 | Tensile strength, lbs. per sq.<br>in.        | 34,000                          | 35,700                       | 38,700                         |
|    | Brinnell hardness No.                        | 196                             | 212                          | 235                            |

The usefulness and value of this new alloy in regular foundry practice are demonstrated by the results given in this table. Its use is not necessarily confined to cast iron, but obviously can be extended to include any metal or alloy in which additions of chromium, titanium, and silicon may be desired, such as steel, nickel, aluminum, or alloys of nickel, copper, etc.

I claim as my invention:

1. An alloy of chromium and titanium for 10 metallurgical use having the approximate composition range: 10 to 30% titanium, 15 to 45% chromium, 20 to 45% silicon, 0.1 to 25% iron, 0.1 to 3% aluminum, 0.01 to 1% carbon, and not over 5% of other impurities.

2. A chromium-titanium-silicon alloy consisting of about 30% chromium, 20% titanium, 35% silicon, 12% iron, 0.1 to 3% aluminum and 0.01 to 1% carbon.

3. A chromium-titanium-silicon alloy consisting of about 30% chromium, 20% titanium, 35% silicon, 12% iron, 0.4% carbon, 1% aluminum, and 1.6% other impurities.

4. A chromium-titanium-silicon alloy consisting of about 27% chromium, 23% titanium, 34% silicon, 14% iron, 1% aluminum, 0.40% carbon and 0.60% other impurities.

GEORGE F. COMSTOCK.